

# UNITED STATES PATENT OFFICE.

GABRIEL VAN OORDT, OF BASEL, SWITZERLAND, ASSIGNOR TO SOCIETE ANONYME DES  
USINES GIULINI, OF BASEL, SWITZERLAND.

PROCESS FOR INCREASING THE HARDNESS AND TENACITY OF METALS AND THE EASE  
OF THEIR WORKING WITH CUTTING-TOOLS.

Specification of Letters Patent. Patented Dec. 30, 1919.

1,326,775.

Application filed April 30, 1919. Serial No. 293,883.

No Drawing.

To all whom it may concern:

Be it known that I, GABRIEL VAN OORDT, Phil. Dr., a subject of the Queen of the Netherlands, and resident of Basel, Switzerland, have invented a new and useful Process for Increasing the Hardness and Tenacity of Metals and the Ease of Their Working with Cutting-Tools, of which the following is a full, clear, and exact specification.

10 It is known that the properties of metals which are technically important can be influenced profoundly by heating the metal to a high temperature.

15 The principle underlying the present invention differs from that underlying the known processes for increasing the hardness and tenacity of metals and the ease of their working with cutting tools that by the invention metals and alloys, particularly 20 aluminium and aluminium alloys are heated, not to high temperatures, but to relatively low temperatures, which are below the characteristic annealing temperatures of the metal in question that is to say the 25 temperatures used for the annealing by heat treatment. The temperature to be used at which a hardness and a tenacity as great as possible are obtained in the shortest time is another for each metal or alloy, but an entirely determined one. This temperature 30 may be called the characteristic heat hardening temperature and is ascertained experimentally.

35 By the invention metals which are worked with difficulty on the lathe are converted in a short time into metals which can be satisfactorily turned and have high tenacity and hardness. By heating to a relatively low temperature there is obtained in the metal, 40 in a very short time, a stable structural equilibrium for the limits of the usual temperatures at which the metal is used.

45 The temperature of the heating is ascertained experimentally by subjecting the metal for a period of several days to a constant temperature and then making hardness tests at room temperature which clearly show whether hardening or softening has occurred. According to the indication thus 50 obtained a further experiment at another, higher, temperature is undertaken and another hardness test made. By the systematic choice of temperatures, one can start from

a low or a high temperature and by gradually raising or lowering the temperature 55 can ascertain that at which hardness is most rapidly acquired. If the hardening experiments for finding out the most advantageous hardening temperature of a metal are extended over a sufficiently long time, that is to 60 say, over about several weeks, the results obtained will show which is the highest hardness obtainable for the metal in question. By varying the temperatures, there is then 65 determined the temperature at which this maximum hardness is the most quickly attained. This temperature is that which is termed the characteristic heat hardening temperature.

70 The object of the invention may, however, also be attained by heating the metal at a temperature below the characteristic heat hardening temperature until the desired hardness has been attained. If the temperature used is not far below the characteristic 75 heat hardening temperature, it is generally possible by longer heating to obtain the maximum hardness of the metal in question. At still lower temperatures, however, this maximum hardness is no longer obtainable 80 but only a hardness smaller than the said maximum hardness. The hardnesses attainable are to a certain extent proportional to the decrease of the hardening temperatures.

85 By a modification of the invention, therefore, there is produced only a partial hardening. This is sufficient when, for example, the main object is to obtain a satisfactory metal for turning or similar working and not a metal having the maximum hardness and 90 tenacity. In such a case the metal part to be hardened may, immediately after casting or reheating in a liquid bath, be brought into a soaking pit or soaking box, which by the heat contained in the metal part is brought 95 to a certain temperature below the characteristic heat hardening temperature; in this pit or box the metal part is left to acquire the desired hardening. The advantage of this form of the invention is that fuel which 100 must be used for the complete heat hardening, can be economized. At the low temperatures used it may not be necessary to protect the metal during heat treatment 105 from atmospheric air by using an indifferent atmosphere or a packing.

By another modification of the invention the hardening operation may be interrupted before the maximum hardness is attained so as to produce a condition in which the metal can be worked with cutting tools and the finished article may be then further subjected to the hardening operation. Such an interruption of the heating for the interpolation of a working operation may be several times repeated and the heating finally carried completely or in part to a finish. For example a screw thread may be cut on the preliminarily hardened metal when the hardening produced is sufficient for the work and then the finished screw can be still further hardened. In this manner the possible softening by strongly heating of the worked surface may be rectified by a subsequent finishing hardening.

20 A partial hardening of metal parts, for instance the hardening of the teeth of toothed wheels, may be simply performed by bringing the parts in question, such as the teeth, to the characteristic heat hardening temperature or a temperature near the said heat hardening temperature, but below it, and cooling when operating on small pieces of the other parts. The parts close to those to be hardened will then have the low temperature at which in the same period the higher or maximum hardness is not attained, so that the hardened parts, for instance the teeth, will be harder than the rest.

25 The metals to employ for toothed wheels are chosen according to the small wear of these latter and to the tenacity necessary for the same and show generally a Brinell hardness of 80 to 100°. The hardening of the teeth of a toothed wheel can for instance be produced by moving the said teeth through an oil bath heated to the characteristic heat hardening temperature. The heat flux through the middle part of the toothed wheel toward the wheel shaft, which moreover can be cooled, is sufficient to produce the necessary decreasing of temperature from the teeth toward the wheel middle to insure a delay in the hardening of the wheel body relative to the hardening of the teeth.

30 In every case, the cooling of the metal from the heat hardening temperature to the ordinary temperature has no influence on the hardness and tenacity of the metal. The metal can therefore be quenched or allowed to cool slowly.

The following examples illustrate the invention:

Example 1: To produce in a piece of alloy consisting of 85 per cent. of aluminium and 15 per cent. of zinc the maximum Brinell hardness of 85.7-92.6, the piece while it is still warm, after having been cast or annealed at 530 to 550° C. if it was previously subjected to a mechanical working in a cold condition, is left for four to five days at a

temperature of about 70° C. either in the air or with exclusion of air, for instance in a partial vacuum or an indifferent atmosphere or in a packing of kieselguhr or clay. The increase of hardness amounts to 80-90 per cent.

The characteristic heat hardening temperature of 70° C. of the alloy employed in this example was determined in the following manner:

After its casting the alloy of 85 per cent. of aluminium and 15 per cent. of zinc was let to cool down in the air. The hardness test made according to Brinell's process with a ball of 10 mm. of diameter and a test pressure of 150 kg. showed for the alloy the hardness of 50 degrees Brinell measured immediately after cooling. Four pieces of this alloy were then subjected to heat treatments at different temperatures, as for instance piece No. 1 at 40° C., piece No. 2 at 70° C., piece No. 3 at 90° C., and piece No. 4 at 110° C.

The heat treatments were interrupted frequently, the metal pieces cooled to room temperature and subjected in every case to a hardness test. The variations of the hardness in each of the four pieces are shown in the following tabular exhibit:

| Test-piece No. | Temper-ature. | Brinell hardness (P=150 kg. and D=10 mm.) after— |           |         |         |         |          |          |          | 100  |
|----------------|---------------|--------------------------------------------------|-----------|---------|---------|---------|----------|----------|----------|------|
|                |               | 9 hours.                                         | 24 hours. | 3 days. | 4 days. | 5 days. | 10 days. | 20 days. | 30 days. |      |
| 1.....         | 40° C.        | 53.4                                             | 60.5      | 69.1    | 74.1    | 79.6    | 85.7     | 85.7     | 85.7     | 85.7 |
| 2.....         | 70° C.        | 60.5                                             | 69.1      | 79.6    | 85.7    | 92.6    | 92.6     | 92.6     | 92.6     | 92.6 |
| 3.....         | 90° C.        | 60.5                                             | 74.1      | 69.1    | 64.6    | 64.6    | 60.2     | 60.2     | 58.3     | 58.3 |
| 4.....         | 110° C.       | 58.6                                             | 64.6      | 69.1    | 69.1    | 69.1    | 64.6     | 64.6     | 56.5     | 56.5 |

This tabular exhibit shows clearly that an alloy of 85 per cent. of aluminium and 15 per cent. of zinc attains the most quickly its maximum hardness by treating it at 70° C. for 4 to 5 days. The increase of hardness amounts to 92.6-50=42.6° Brinell that is to say 85 per cent. of the initial hardness.

If after casting the alloy was subjected to a mechanical working, as rolling, drawing or hammering, an annealing of the metal at 530° to 550° followed by a cooling down in the air had to take place before its heat treatment at 70° C.

Before its hardening the alloy showing a Brinell hardness of 50° could difficultly be worked with cutting tools. After its hardening to 92.6° Brinell it could be turned on the turning lathe as easily as brass. After its hardening the alloy had not lost its ductility and could further be worked mechanically by rolling, drawing, etc. at room temperature, producing thus a further increase of hardness and tenacity and ease of working with cutting tools. It is necessary that such a mechanical working after the heat

hardening be effected at a temperature below 70° C. that is to say below the characteristic heat hardening temperature and it is therefore convenient to cool the metal frequently during the mechanical working.

Example 2: For attaining the highest Brinell hardness of 55.3 a piece of alloy consisting of 98 per cent. aluminium and 2 per cent. copper, while it is still warm after casting or annealing, is warmed for 10 days to about 160° C., in air or with exclusion of air as described in Example 1. By this treatment the hardness of this alloy is increased by about 70 per cent., the initial 15 hardness having been 32.7 degrees Brinell.

The following tabular exhibit shows how the characteristic heat hardening temperature was determined:

| 20 | Test-piece No. | Temperature. | Brinell hardness (P=150 kg. and D=10 mm.) after— |          |        |        |         |         |         |
|----|----------------|--------------|--------------------------------------------------|----------|--------|--------|---------|---------|---------|
|    |                |              | 9 hours                                          | 24 hours | 3 days | 5 days | 10 days | 20 days | 30 days |
| 25 | 1              | 35° C.       | 32.7                                             | 35.7     | 35.7   | 35.7   | 37.2    | 39.0    | 39.0    |
|    | 2              | 65° C.       | 32.7                                             | 35.7     | 35.7   | 37.2   | 42.9    | 42.9    | 42.9    |
|    | 3              | 105° C.      | 32.7                                             | 35.7     | 35.7   | 37.2   | 42.9    | 46.3    | 52.4    |
|    | 4              | 160° C.      | 32.7                                             | 35.7     | 39.0   | 42.9   | 55.3    | 55.3    | 55.3    |
|    | 5              | 190° C.      | 32.7                                             | 35.7     | 42.9   | 42.9   | 39.0    | 37.1    | 35.0    |

30 After 10 days the maximum hardness of 55.3 was consequently attained.

While for aluminium and its alloys with preponderating aluminium content the so-called heat hardening temperature amounts to at most about 160–200° C., this temperature for metals, such as copper, brass, bronze or the like is much higher correspondingly with their higher melting points.

Example 3: By heating pure zinc for 24 hours at about 300° C. the highest Brinell hardness of 39.0 is attained, which is an increase of hardness of about 10 per cent. of that of the unhardened zinc.

Example 4: Pure copper having a Brinell hardness of 30° acquires the highest Brinell hardness of 42.9 in 20 days at a temperature of about 200° C., the increase of hardness being about 40 per cent.

The determination of the characteristic heat hardening temperature of 200° C. resulted from the experiments shown in the following tabular exhibit:

| 65 | Test-piece No. | Temperature. | Brinell hardness (P=150 kg. and D=10 mm.) after— |          |        |        |         |         |         |
|----|----------------|--------------|--------------------------------------------------|----------|--------|--------|---------|---------|---------|
|    |                |              | 9 hours                                          | 24 hours | 3 days | 5 days | 10 days | 20 days | 30 days |
| 60 | 1              | 110° C.      | 30.0                                             | 30.3     | 32.5   | 32.5   | 32.5    | 32.5    | 32.5    |
|    | 2              | 160° C.      | 30.0                                             | 32.7     | 32.7   | 32.7   | 32.7    | 32.7    | 42.7    |
|    | 3              | 200° C.      | 31.2                                             | 32.7     | 32.7   | 35.7   | 35.7    | 39.0    | 42.9    |
|    | 4              | 300° C.      | 31.2                                             | 31.2     | 32.7   | 35.7   | 35.7    | 39.0    | 38.0    |

Example 5: In 5 days the Brinell hardness of bronze of the composition 94 per cent. copper and 6 per cent. tin is increased

to 65.5 by heating at a temperature of 500° C. The increase of hardness is about 12 per cent.

Example 6: Heating brass of the composition 72 per cent. copper and 28 per cent. zinc at about 300° C. for 3 days, increases the 70 Brinell hardness to 47.4, that is to say about 15 per cent.

Example 7: A soft iron having a Brinell hardness 85.7 has this hardness increased to 104 by a heating for about 50 days at 300° C. 75 The heating should be conducted in an indifferent atmosphere or in a packing or in some other manner excluding air. The increase of hardness amounts to 21 per cent. After 10 days the hardness was 92.6 and 80 after 15 days 100 on the same scale.

The following tabular exhibit shows how the characteristic heat hardening temperature of 300° C. has been determined:

| Test-piece No. | Temperature. | Brinell hardness (P=150 kg. and D=10 mm.) after— |        |        |         |         |         |         |
|----------------|--------------|--------------------------------------------------|--------|--------|---------|---------|---------|---------|
|                |              | 1 day                                            | 3 days | 5 days | 10 days | 15 days | 30 days | 50 days |
| 1              | 150° C.      | 85.7                                             | 85.7   | 85.7   | 85.7    | 85.7    | 85.7    | 85.7    |
| 2              | 260° C.      | 85.7                                             | 85.7   | 85.7   | 89.0    | 89.0    | 89.0    | 89.0    |
| 3              | 300° C.      | 85.7                                             | 85.7   | 85.7   | 92.0    | 92.6    | 100     | 104     |
| 4              | 380° C.      | 85.7                                             | 85.7   | 89.0   | 89.0    | 89.8    | 89.8    | 89.8    |

Example 8: Metal parts consisting of 95 per cent. aluminium and 15 per cent. zinc were warmed at about 40° C. for 4 days and thereby attained Brinell hardness of 74.1 corresponding with an increase of hardness of 56 per cent. 10 days' heating at the same 100 temperature raised the hardness to 85.7 Brinell, an increase of 80 per cent. and this was the maximum result of this particular heat hardening (the characteristic heat hardening temperature is about 70° C.).

Example 9: A piece of metal consisting of 98 per cent. aluminium and 2 per cent. copper attains a Brinell hardness of 42.9 when heated for 10 days at about 120° C. corresponding with an increase of hardness 110 of about 28 per cent. The like treatment for 25 days produced the maximum Brinell hardness of 55.3 degrees. (The characteristic heat hardening temperature is about 160° C.).

Example 10: Pure zinc heated for 2 days at about 200° C. yielded the maximum Brinell hardness of 39, an increase of hardness of 10 per cent. The like heat treatment for 20 hours only produced an increase of hardness of 6 per cent. or 37.8 Brinell hardness. 115 (The characteristic heat hardening temperature is about 300° C.).

Example 11: At 210° C. a brass consisting of 72 per cent. copper and 28 per cent. zinc can be brought in 10 days to a Brinell hardness of 45 degrees, the increase of hardness being of about 5 per cent. (The characteristic heat hardening temperature is about 300° C.).

Example 12: Heating at 260° C. for 10 130

days increases the hardness of soft iron by about 4 per cent. (The characteristic heat hardening temperature is about 300° C.).

The heat hardening treatment may be applied to the finished product or may be interposed intelligently between the stages of working of the process to which the metal is subjected. The heat hardening however, cannot be followed by any mechanical working by means of presses, rollers, hammers or the like at temperatures higher than the characteristic heat hardening temperature. On the other hand permissible cold working by means of presses, rollers, hammers, drawings etc. produces a further increase of hardness, tenacity and ease of working with cutting tool.

What I claim is:

1. The herein described process for increasing the hardness, and tenacity of metals and the ease of their working with cutting tools, consisting in heating the metal to a relatively low temperature which is below the characteristic temperature for the annealing of the metal in question.
2. The herein described process for increasing the hardness of aluminium and aluminium alloys having a preponderating aluminium content, which consists in heating the metal or alloy at a temperature between 160° and 200° C. until maximum hardness is attained.
3. The herein described process for increasing the hardness, and tenacity of metals and the ease of their working with cutting

tools, consisting in heating the metal to its characteristic heat hardening temperature or to a temperature below this characteristic heat hardening temperature until the desired hardness has been attained.

4. The herein described process for increasing the hardness, and tenacity of metals and the ease of their working with cutting tools, consisting in heating the metal to its characteristic heat hardening temperature or to a temperature below this characteristic heat hardening temperature, interrupting the heat hardening before the attainment of the final condition, then working the metal with a cutting tool and then continuing the heat hardening until the desired or maximum hardness has been attained.

5. The herein described process for increasing the hardness, and tenacity of metal articles and the ease of their working with cutting tools, consisting in heating certain parts of the article to the characteristic heat hardening temperature or a temperature near the said heat hardening temperature, but below it, while the other parts of the article are kept at a lower temperature, until the parts to be hardened have attained the maximum or desired hardness.

In witness whereof I have hereunto signed my name this 14th day of April, 1919, in the presence of two subscribing witnesses.

DR. GABRIEL VAN OORDT.

Witnesses:

SCOTT TAGGART,  
ARNAUD BRAM.